

July 9, 1946.

E. E. JELLEY ET AL

2,403,721

PREVENTING COLOR FOG IN PHOTOGRAPHIC MATERIAL

Filed Sept. 23, 1943



EDWIN E. JELLEY  
PAUL W. VITTM

INVENTORS

BY *Newton M. Perrine*  
*R. Frank Smith*  
ATTORNEYS

## UNITED STATES PATENT OFFICE

2,403,721

## PREVENTING COLOR FOG IN PHOTOGRAPHIC MATERIAL

Edwin E. Jelley and Paul W. Vittum, Rochester, N. Y., assignors to Eastman Kodak Company, Rochester, N. Y., a corporation of New Jersey

Application September 23, 1943, Serial No. 503,472

5 Claims. (Cl. 95—8)

1

This invention relates to color photography and particularly to a method for preventing the formation of color fog or stain in photographic emulsions containing couplers.

The method of color photography in which color-forming or coupling compounds combine with the development product of aromatic amino photographic developers to produce dyes is well known. The color formers or couplers used in this method may be added directly to the sensitive emulsion layers as described in Fischer U. S. Patent 1,102,028, granted June 30, 1914, or may be incorporated in a water-permeable medium which is insoluble in the colloidal carrier for the sensitive silver salt as described in Mannes & Godowsky U. S. Patent 2,304,940, granted December 15, 1942, or our U. S. Patent 2,322,027, granted June 15, 1943.

A difficulty frequently encountered in these processes is the formation of color fog or stain. When the exposed material is developed in a color-forming developer, dye fog is frequently formed in the emulsion layer. This is because the developing agent has been oxidized to some extent by the action of the air and the oxidized developer tends to couple with the color-forming compound at places in the photographic material where no silver image is produced. It is well known that in these processes the dye should be formed only where the silver halide is reduced to metallic silver, thereby oxidizing the developing agent to a form which couples with the color former. Once the developing agent is oxidized, it couples immediately with the color former whether a photographic image is present or not. Aerial oxidation of the developer or oxidation by means other than the photographic image therefore converts the developer to a form which will immediately react with the color former to produce a color fog or stain. This effect is especially noticeable in materials having couplers incorporated in the sensitive emulsion layer since there is no coupler in the developing solution to react with any developing agent which is oxidized by the action of the air. Fog or stain arising from these causes is not readily controlled by the same procedures used to control silver fog.

It is an object of the present invention to prevent that particular type of color fog which is caused by the oxidized developer penetrating the upper layers of a multilayer photographic material containing couplers. A further object is to provide a sensitive photographic material containing couplers and provided with an overcoating layer which affords protection against such fog.

These objects are accomplished, according to our invention, by providing over the multilayer material a layer of a water-permeable colloidal material containing a substantially non-diffusing

5

reducing agent capable of reacting with the oxidized developer in the developing solution to yield substantially colorless products. The oxidized developer present in the developing solution is thereby prevented from reaching the sensitive layers containing couplers and combining with the couplers where the layer was not exposed. The unoxidized developing agent can penetrate through the layer containing the reducing agent unaffected, and develop the exposed portions of the emulsion layer or layers to form colored images therein.

10

In the accompanying drawing the single figure is a sectional view of a film constructed according to our invention.

15

The water-permeable layer containing the reducing agent used according to our invention is coated over the sensitive emulsion layer of the photographic material. The overcoating layer may be used with single layer photographic materials although it is of greater value with multilayer materials containing couplers in one or more of the sensitive emulsion layers such as those described in the Mannes & Godowsky U. S. Patent 2,304,940 or our U. S. Patent 2,322,027, referred to above. The sensitive material may be film or paper and may have a transparent or an opaque base.

20

In the case of a film material, the effect of the extra layer containing the reducing agent is to render the developer diffusing through it substantially free from oxidation products which would otherwise cause color fog. With paper materials, most of the diffusion takes place through the emulsion side so that the overcoating layer is usually adequate for preventing stain. However, there might be a slight gain in freedom from color fog in the lowermost sensitive layer of a paper coating if a layer were placed between it and the paper base containing a substantially non-diffusing reducing agent capable of destroying developer oxidation products.

25

The overcoating layer used according to our invention may consist of any suitable water-permeable colloidal material such as gelatin, collodion or other cellulose ester or synthetic resin such as polyvinyl alcohol. A suitable amount of a reducing agent is added to the colloidal material which is coated as a layer on the finished film. The reducing agent should be non-diffusing in the layer in which it is incorporated so that it does not contaminate the adjacent sensitive emulsion layer. We prefer to use an organic reducing agent containing an aliphatic group having a carbon chain of at least 8 carbon atoms, such as a higher fatty acid residue. Hydroquinones having long chain aliphatic groups are especially suitable although we may also use p-aminophenols, hydrazines or ascorbic acid derivatives.

2

30

35

40

45

50

55

60

The following compounds, which are by way of example only, are suitable for use according to our invention:



n-Octyl hydroquinone



Di-n-octyl hydroquinone



n-Dodecyl hydroquinone



Di-n-dodecyl hydroquinone



Octadecyl hydroquinone



Chloro-n-dodecyl hydroquinone



Lauryl gentisate



2-lauroylamino-4-aminophenol



p-Laurylphenylhydrazine

The reducing agents for lowering color fog may be incorporated directly in the gelatin or other colloidal material of the overcoating layer or may be incorporated in a water-permeable, water-insoluble vehicle which is dispersed in the gelatin or other colloidal carrier. The method of incorporating the reducing agent will be explained by reference to the following examples.

## Example 1

A solution of 2 grams of didodecyl hydroquinone in a mixture of 130 cc. of 95% ethyl alcohol and 10 cc. of 20% sodium hydroxide solution was added to 1000 cc. of melted 5% gelatin solution. To this solution there was added sufficient citric acid solution to bring the pH to the desired value, for example, about pH 6.5. The mixture was then coated on a multilayer material containing couplers.

## Example 2

A solution containing 4.5 grams of p-lauryl phenyl hydrazine and 10 grams of n-butylphthalate in 200 cc. of ethyl acetate was emulsified with 400 cc. of 0.5% aqueous solution of triisopropyl naphthalene sulfonate. The emulsification was effected by passing the mixture several times through a colloid mill. The resulting emulsion was subjected to heating on a steam bath with constant stirring to dissolve off the ethyl acetate and the remaining water suspension was added to 500 cc. of melted 10% gelatin. This mixture was diluted with water to one liter and was then coated on a multilayer material containing couplers.

Our invention will now be described by reference to the accompanying drawing.

As shown in the drawing, which is a sectional view of a film constructed according to our invention, 10 is a support of cellulose ester or other suitable material having thereon gelatino-silver halide emulsion layers 11, 12 and 13 sensitive, respectively, to the red, green and blue regions of the spectrum. Emulsion layer 11 contains a coupler capable of producing a cyan dye image upon development, emulsion layer 12 contains a coupler capable of producing a magenta dye image upon development, and emulsion layer 13 contains a coupler capable of producing a yellow dye image upon development. Suitable couplers are described in Mannes & Godowsky U. S. Patent 2,304,940 or our U. S. Patent 2,322,027. The usual yellow filter layer 14 is employed between layers 12 and 13 to prevent action of blue light on the layers 11 and 12. Over the layer 13 there is a gelatin layer 15 containing a reducing agent which is non-diffusing in the gelatin.

In our process the reducing agent is located in its own separate layer away from the sensitive silver halide. For this reason, together with the fact that the reducing agent is substantially non-diffusing, agents may be used which could not be added to an emulsion layer because of fogging, desensitizing or interfering with normal dye-image formation.

The reducing power of the reducing agents used, according to our invention, may be determined by reference to their action on a solution of ammoniacal silver nitrate. A solution of ammoniacal silver nitrate is prepared by making a  $\frac{1}{2}$  normal solution of silver nitrate and adding to it a 28% solution of ammonium hydroxide slowly until the first formed precipitate just dissolves. The compound to be tested for determining its suitability for use in our invention is

then added to the ammoniacal silver nitrate solution. If it reduces the silver nitrate immediately and without heating, to metallic silver, it is suitable for use according to our invention.

It will be understood that the examples and modifications included herein as by way of example only and that our invention is to be taken as limited only by the scope of the appended claims.

We claim:

1. A multilayer photographic film comprising a support having thereon at least one silver halide emulsion layer containing a coupler, and over said emulsion layer an outermost, exposed layer of a water-permeable colloid containing an organic reducing agent for oxidized photographic developers, said reducing agent containing an aliphatic group having a carbon chain of at least 8 carbon atoms and being non-diffusing in said water-permeable colloid layer.

2. A multilayer photographic film comprising a support having thereon at least one silver halide emulsion layer containing a coupler, and over said emulsion layer a layer of a water-permeable colloid containing a hydroquinone having attached thereto a substituent group rendering said

hydroquinone non-diffusing in said water-permeable colloid layer.

3. A multilayer photographic film comprising a support having thereon at least one silver halide emulsion layer containing a coupler, and over said emulsion layer a layer of a water-permeable colloid containing a hydroquinone having therein an aliphatic group having a carbon chain of at least 8 carbon atoms.

10 4. A multilayer photographic film comprising a support having thereon at least one gelatino-silver halide emulsion layer containing a coupler, and over said emulsion layer a layer of gelatin containing a hydroquinone having therein an aliphatic group having a carbon chain of at least 8 carbon atoms.

5. A multilayer photographic film comprising a support having thereon at least one gelatino-silver halide emulsion layer containing a coupler, and over said emulsion layer a layer of gelatin containing a hydroquinone substituted with an alkyl radical having a carbon chain of at least 8 carbon atoms.

EDWIN E. JELLEY.

PAUL W. VITTUM.